

## UNITED STATES PATENT OFFICE

1,984,303

## MANUFACTURE OF ARTIFICIAL SILK

Gustav Hardt, Elizabethton, Tenn., assignor to  
American Bemberg Corporation, New York,  
N. Y., a corporation of Delaware

No Drawing. Application October 4, 1932,  
Serial No. 636,177

7 Claims. (Cl. 106—40)

My present invention has to do with a new and novel method for producing artificial cellulosic products with a low lustre.

More especially, my present invention concerns a new method for producing artificial filaments which possess the desirable low lustre of real silk.

One object of the present invention is to provide a novel method for producing a filament or thread of artificial silk which has greater opacity and covering power, and which possesses a low or dull lustre.

Other objects will become apparent from a study of the following specification and claims.

In the manufacture of artificial filaments, a cellulosic solution is prepared (cuprammonium, viscose, nitrocellulose or organic derivatives of cellulose), and spun or extruded into a medium which tends to harden the filaments thus formed. My present invention has to do with a new and novel mixture or compound, to be added to the spinning solution before the filaments are formed, and which remains in the filaments during the after treatment thereof. The presence of this substance in the filaments gives them the greater opacity and covering power desired and renders them lustreless.

I prepare an emulsion of certain compounds and add this emulsion to the spinning solution prior to the formation of filaments therefrom. The ingredients of my emulsion include a phosphorprotein such as casein, paracasein and vitellin. Casein is well known as the chief nitrogenous constituent of milk, and is found dissolved therein in the form of a salt containing the percentage composition of a protein with approximately 0.85 percent of phosphorous. Another of the ingredients of my emulsion is petrolatum. The two remaining constituents are oleic acid and triethanolamine, the latter having the formula  $(\text{CH}_2\text{OHCH}_2)_3\text{N}$ .

These constituents need not all be used together, since the petrolatum may or may not be present. I have found, however, that the presence of petrolatum tends to produce a filament with a duller lustre.

As examples of my new invention, the following are given. All percentages are calculated on the cellulose content of the solution.

Example A.—A cellulosic spinning solution is

prepared in the usual manner, and to this is added, in an emulsified form, a compound of the following composition:

|                 |        |                      |   |
|-----------------|--------|----------------------|---|
| Casein          | 10.00% | (based on cellulose) | 5 |
| Petrolatum      | 10.00% | (based on cellulose) |   |
| Oleic acid      | 13.00% | (based on cellulose) |   |
| Triethanolamine | 0.45%  | (based on cellulose) |   |

Example B.—A spinning solution is made up, as in Example A, and to this is added, as an emulsion:

|                 |        |                      |    |
|-----------------|--------|----------------------|----|
| Casein          | 10.00% | (based on cellulose) | 10 |
| Oleic acid      | 10.00% | (based on cellulose) |    |
| Triethanolamine | 0.45%  | (based on cellulose) | 15 |

The solution is thoroughly mixed, in each case, before spinning.

Having now set forth my invention as required by the patent statutes, what I desire to claim is:

1. A cellulose filament, containing a phosphorprotein, oleic acid and triethanolamine. 20

2. A spinning solution for the manufacture of artificial products comprising a cellulosic spinning solution, a phosphor protein, oleic acid and triethanolamine. 25

3. A spinning solution for the manufacture of artificial products comprising a cellulosic spinning solution, casein, oleic acid and triethanolamine. 30

4. A spinning solution for the manufacture of artificial products comprising a cellulosic spinning solution, a phosphor protein, oleic acid, petrolatum and triethanolamine. 35

5. A spinning solution for the manufacture of artificial products comprising a cellulosic spinning solution, casein, oleic acid, petrolatum and triethanolamine. 40

6. A spinning solution for the manufacture of artificial products comprising a cellulose spinning solution, about 10% casein, about 10% oleic acid and about 0.45% triethanolamine, said percentages being based upon the cellulose content of said spinning solution. 45

7. A cellulosic spinning solution for the manufacture of artificial products comprising a cellulosic spinning solution, about 10% casein, about 10% petrolatum, about 13% oleic acid and about 0.45% triethanolamine, said percentages being based upon the cellulose content of said spinning solution. 50

GUSTAV HARDT. 50